

## UNITED STATES PATENT OFFICE

2,288,289

## LUBRICANT

Bert H. Lincoln, Gordon D. Bykit, and Waldo L. Steiner, Ponca City, Okla., assignors, by mesne assignments, to Socony-Vacuum Oil Company, Incorporated, New York, N. Y., a corporation of New York

No Drawing. Application April 17, 1940,  
Serial No. 330,684

6 Claims. (Cl. 252—35)

Our invention relates to improved lubricants and more particularly to lubricants containing in combination an addition agent, giving the finished composition increased resistance to oxidation and the formation of corrosive products as well as other improved characteristics.

This is a continuation-in-part of our co-pending application, Serial No. 223,070, filed August 4, 1938.

Modern mechanical devices require lubricating oils of high film strength, high oiliness characteristics, and oxidation-resisting characteristics. Straight hydrocarbon lubricants including high quality, highly refined hydrocarbon oils are deficient in these three important characteristics. Oiliness properties, film strength, and resistance to oxidation are of vital importance under conditions of boundary or thin film lubrication in which the lubricating film has been squeezed between two moving surfaces by pressure. The importance of these three characteristics is magnified with large bearing surfaces and slow speeds.

It will be clear to those skilled in the art that the viscosity of a lubricant plays no part in these characteristics. A high-quality paraffin base Pennsylvania lubricating oil would still fail if deficient in film strength as a rupture of the film would permit metal-to-metal contact and resulting injury or seizure. The oil film, lacking in oiliness qualities, imparts resistance to movement. In many conditions of use, the oil must resist oxidation from atmospheric oxygen.

The present-day trend in internal combustion engines to high compression ratios requires the use of higher film strength lubricants, and it has been found that even the best quality hydrocarbon oil possesses a film strength too low to enable it to lubricate satisfactorily.

Many mechanical devices operate frequently under conditions of boundary or thin film lubrication. Under these conditions, the oiliness, the film strength, and the resistance to oxidation become most important.

The oxidation of lubricating oil hydrocarbons results in the formation of compounds which polymerize or sludge. Acids are formed which are especially deleterious under conditions of thin film lubrication. The acid, too, has an especially adverse effect on modern bearing compositions such as cadmium-silver and copper-lead. The sludge formed has no lubricating properties, and even the best hydrocarbon lubricant will be quickly deteriorated if subjected to oxidation conditions.

In those devices in which a lubricant is cir-

culated by means of a pump, there is usually a short period when the devices started from a condition of rest in which the surfaces operate under conditions of substantially dry friction, if ordinary hydrocarbon lubricants are used. It will be readily apparent to those skilled in the art that with dry friction the wear on the friction surfaces is extreme. This condition is magnified during cold weather when the viscosity of the lubricant is high and the oil circulation is slow. An accident to the oil circulation system invariably spells disaster with ordinary hydrocarbon lubricants.

In the prior art, it has been the practice to refine an oil thoroughly by means of acid or selective solvent treatments. This drastic refining has been necessary in order to remove unstable compounds which will polymerize or sludge. The refined oil, however, appears to be more readily oxidizable than an unrefined oil, with the result that a highly refined oil will quickly oxidize and form soluble acids and other corrosive materials. Highly refined oils, upon oxidation, also form lacquer-like polymers which tend to cause sticking of the piston rings. This sticking in an internal combustion engine results in loss of power, failure of lubrication, scratching, scoring, overheating, and eventually failure of parts, necessitating replacement. It is practically impossible to refine a lubricant in such a manner as to avoid all three of these difficulties, namely, slugs, soluble corrosive products, and lacquer.

The trend of development in internal combustion engines has imposed increasing burdens upon the oils used for their lubrication, particularly with respect to operating temperatures and pressures. At present, the Diesel type of engine probably represents extreme requirements in both of these respects; but it is not alone in the imposition of severe burdens upon the lubricating oil used. The useful operating life of a lubricating oil, in such service, is determined, in large measure, by its thermal stability and by its physical capacity to continue functioning as a lubricant, at the high temperatures and high pressures encountered. One measure of thermal stability is resistance to oxidation, and the consequent tendency to form sludge; but in another aspect the effect of thermal instability is determined not only by the extent of oxidation or decomposition but also by the character of the products of such decomposition or oxidation and by the extent and location, within the engine, of deposits of such products.

In the Diesel type of engine, the high temperatures to which the lubricating oil is subjected, particularly at the top of the stroke, frequently cause deposition of sludge and carbon in the groove for and behind one or more of the piston rings. Using paraffinic type lubricating oils, such difficulties are usually more pronounced with respect to the uppermost ring; using naphthenic type lubricating oil, they are usually more pronounced with respect to the lower rings. Consequent sticking of the rings rapidly deprives the piston and cylinder wall of proper lubrication, inducing wear and, frequently, scoring of the cylinder wall. The formation of such "carbon" deposits, hard enough and coherent enough to involve sticking of the rings, is materially retarded, if not avoided, by the use of the improved lubricating oil compositions of our invention; and in this aspect the self-cleaning properties of the lubricating oil compositions of our invention, with respect to the engine, make a mere change of oil a substitute, economical with respect both to loss of service time and cost, for many otherwise necessary cleaning and repair jobs.

One object of our invention is to provide a lubricant which has the important property of reacting with metal surfaces, penetrating or being adsorbed on the metal surfaces in order to leave at all times a film of lubricant of high oiliness character which will remain on the metal surfaces irrespective of the length of time the machine or device has been idle.

Another object of our invention is to provide a lubricant of high oiliness properties so that the lubricating film will give a very smooth and even operation.

Another object of our invention is to provide a hydrocarbon lubricant which, when diluted with unburned fuel or with other light hydrocarbons, reducing the viscosity, will nevertheless have such a degree of oiliness and film strength as to offset the dilution without impairing the load-carrying ability of the lubricant.

Another object of our invention is to provide a lubricant which is effective in highly refined, poorly refined, or even wholly unrefined lubricants, which will provide the finished composition with marked anti-sludging, increased film strength, and high oiliness characteristics.

Another object of our invention is to provide lubricants containing added materials which reduce markedly the lacquer and carbon-forming tendencies of the hydrocarbon portion of the lubricant and minimize difficulties due to ring-sticking.

Other and further objects of our invention will appear from the following description.

In general, our invention contemplates the combination of a lubricant containing an oil of lubricating viscosity and an addition agent comprising stannic tin salts or soaps of organic acids containing at least one aromatic nucleus. The hydrocarbon oil, if desired, may be of fuel hydrocarbon oil so that, upon combustion of the fuel, the deposition of the addition agent upon the cylinder walls will result in its becoming admixed with the crankcase lubricant.

By way of illustration and not by way of limitation, some of the particular stannic salts of organic acids containing at least one aromatic nucleus will be mentioned hereinbelow. The aromatic nucleus is essential to provide sufficient stability and solubility in hydrocarbons. Tin stearate, for example, is not suitable in the use

of our invention. It is difficultly soluble in hydrocarbon oils. Tin naphthenate is another example of a compound not falling within the class of the compounds of our invention. It is, compared with our compounds, unstable and does not appear to produce our improved results.

Our compounds are particularly efficient in preventing the development of corrosive materials during use. Some illustrative examples of our stannic salts containing at least one aromatic group and capable of being used in our invention follow. Each of these compounds is disclosed as an example of a lubricant containing the compounds.

15 I. Acid group on aromatic ring

A. Alkylated aromatic acids

1. Stannic p-cetyl benzoate  
(C<sub>12</sub>H<sub>23</sub>C<sub>6</sub>H<sub>4</sub>CO<sub>2</sub>)<sub>4</sub>Sn
2. Stannic tri-isoctylbenzene sulfonate  
(C<sub>12</sub>H<sub>23</sub>)<sub>3</sub>C<sub>6</sub>H<sub>2</sub>SO<sub>3</sub>)<sub>4</sub>Sn

B. Aldehyde acids

1. Stannic salt of the half aldehyde of terephthalic acid  
(H.CO.C<sub>6</sub>H<sub>4</sub>CO<sub>2</sub>)<sub>4</sub>Sn

C. Keto acids

1. Stannic benzophenone-4-carboxylate  
(C<sub>6</sub>H<sub>5</sub>CO.C<sub>6</sub>H<sub>4</sub>CO<sub>2</sub>)<sub>4</sub>Sn
2. Stannic p-lauroylbenzoate  
(C<sub>11</sub>H<sub>23</sub>CO.C<sub>6</sub>H<sub>4</sub>CO<sub>2</sub>)<sub>4</sub>Sn

D. Ether acids

1. Stannic p-amyoxybenzoate  
(C<sub>6</sub>H<sub>11</sub>OC<sub>6</sub>H<sub>4</sub>CO<sub>2</sub>)<sub>4</sub>Sn
2. Stannic p-phenoxybenzoate  
(C<sub>6</sub>H<sub>5</sub>OC<sub>6</sub>H<sub>4</sub>CO<sub>2</sub>)<sub>4</sub>Sn

E. Nitro acids

1. Stannic 1-nitronaphthalene - 2 - carboxylate  
(C<sub>10</sub>H<sub>8</sub>(NO<sub>2</sub>)CO<sub>2</sub>)<sub>4</sub>Sn

F. Amino acids

1. Stannic p-diamylaminobenzoate  
(C<sub>12</sub>H<sub>25</sub>)<sub>2</sub>NC<sub>6</sub>H<sub>4</sub>CO<sub>2</sub>)<sub>4</sub>Sn
2. Stannic chloro-diethylaminobenzoate  
(C<sub>2</sub>H<sub>5</sub>)<sub>2</sub>NC<sub>6</sub>H<sub>3</sub>Cl.CO<sub>2</sub>)<sub>4</sub>Sn

II. Acid group on side chain

A. No substituents on aromatic radical

1. Stannic phenylstearate  
(C<sub>17</sub>H<sub>34</sub>(C<sub>6</sub>H<sub>5</sub>)CO<sub>2</sub>)<sub>4</sub>Sn

B. Alkylated on aromatic radical

1. Stannic tributylphenylacetate  
(C<sub>4</sub>H<sub>9</sub>)<sub>3</sub>C<sub>6</sub>H<sub>2</sub>CH<sub>2</sub>CO<sub>2</sub>)<sub>4</sub>Sn
2. Stannic tetrabutylcinnamate  
(C<sub>4</sub>H<sub>9</sub>)<sub>4</sub>C<sub>6</sub>H<sub>2</sub>CH=CHCO<sub>2</sub>)<sub>4</sub>Sn
3. Stannic tridodecylhydrocinnamate  
(C<sub>12</sub>H<sub>25</sub>)<sub>3</sub>C<sub>6</sub>H<sub>2</sub>CH<sub>2</sub>CH<sub>2</sub>CO<sub>2</sub>)<sub>4</sub>Sn
4. Stannic delta-tributylphenyl-n-valerate  
(C<sub>4</sub>H<sub>9</sub>)<sub>3</sub>C<sub>6</sub>H<sub>2</sub>(CH<sub>2</sub>)<sub>4</sub>CO<sub>2</sub>)<sub>4</sub>Sn
5. Stannic di-isoctylphenylethyl sulfonate  
(C<sub>12</sub>H<sub>23</sub>)<sub>2</sub>C<sub>6</sub>H<sub>3</sub>CH<sub>2</sub>CH<sub>2</sub>SO<sub>3</sub>)<sub>4</sub>Sn

C. Keto acids

1. Stannic-o-butyrophenylacetate  
(C<sub>3</sub>H<sub>7</sub>CO.C<sub>6</sub>H<sub>4</sub>CH<sub>2</sub>CO<sub>2</sub>)<sub>4</sub>Sn

D. Ether acids

1. Stannic beta-ethoxyethylphenylacetate  
(C<sub>2</sub>H<sub>5</sub>OCH<sub>2</sub>CH<sub>3</sub>C<sub>6</sub>H<sub>4</sub>CH<sub>2</sub>CO<sub>2</sub>)<sub>4</sub>Sn
2. Stannic beta-chloroethoxyphenylacetate  
(ClCH<sub>2</sub>CH<sub>2</sub>OCH<sub>2</sub>C<sub>6</sub>H<sub>4</sub>CH<sub>2</sub>CO<sub>2</sub>)<sub>4</sub>Sn

The preparation of some of the acids useful in making these stannic salts is described in U. S. Patent 2,111,820 to Steindorff et al. The stannic salts are made, for example, by treating dilute methanol solutions of the sodium or ammonium salt of the acid with a methanol solution of anhydrous stannic chloride (CnCl<sub>4</sub>) and filtering off

the soap. It may also be separated from the methanol solution by dissolving in a light oil (70 or 150 pale oil). The soap or its oil solution is freed from moisture and methanol by warming under reduced pressure.

Any of the foregoing compounds or other members of the classes represented by them or derivatives of these compounds are within the scope of our invention.

It is to be understood that in practicing our invention, oil-soluble stannic salts of the type described are to be selected. Some of the examples described have only limited solubility in hydrocarbon oils. It is to be remembered, however, that, because of their great efficiency, extremely small amounts are often effective. Thus we may use as little as 0.001 per cent of some of these compounds, and it will be seen that a fairly insoluble material may dissolve to a sufficient extent to be satisfactory for our purpose. In general, 0.001 per cent or more of our addition agents are used; and we may add one, two, or even five per cent or more. Form 0.01 per cent to 1.5 per cent of most of the compounds is usually considered adequate.

Furthermore, it is well known that different types of oils have different capabilities of dissolving a given material. For some purposes, therefore, we prefer paraffinic lubricants; for other purposes, asphaltic lubricants; and for still other purposes, naphthenic or mixed base lubricants. Another method of obtaining a satisfactory mixture of addition agent with the hydrocarbon oil is the use of a mutual solvent to bring the addend into solution. Alternatively, peptizing agents may be added to maintain the stannic salts in permanent suspension.

Many of the more difficultly soluble materials are rendered more soluble by the introduction of alkyl groups, particularly those containing four or more carbon atoms. The isoamyl, cetyl, lauryl, and octadecyl radicals and radicals from paraffin wax greatly increase the solubility of organic compounds in oil. One or more of such groups may be introduced into any of the foregoing compounds, derivatives, or homologues, as required. For example, stannic stearate is not very soluble in hydrocarbon lubricating oils, but stannic phenylstearate is much more soluble; and stannic phenylstearate with a wax radical on the phenyl group is still more soluble.

The selection of a particular compound or compounds to be used as an addition agent to the hydrocarbon oil is to be made considering the physical and chemical properties of the various compounds and the use to which the blend is put.

By oil having lubricating characteristics in the appended claims, we mean to include the so-called mineral oils and various hydrogenated, polymerized, and otherwise synthetically treated oils such as voltolized oils, aluminum chloride treated oils, and the like. Furthermore, the lubricating oil may consist in whole or in part of shale oil or of animal or vegetable oils such as caster oil, lard oil, corn oil, cottonseed oil, and the like.

It is sometimes advantageous to combine more than one of these compounds in a blend to obtain particular properties. We accomplish this by mixing two or more of these compounds together and blending the mixture with the hydrocarbon oil or by blending one in the hydrocarbon oil, blending the second into this mixture, and so on until the composition is complete.

The various stannic salts usually improve both

the film strength and oxidation characteristics of the hydrocarbon oil. For example, the sludging tendencies may be decreased by as little as 0.001 per cent of our tin compounds. The oxidation characteristics of lubricants are very important, and these are markedly improved by our compounds. The ability to reduce friction is another feature contributed to lubricants by some of our tin compounds.

It may be desirable to include in one and the same blend, in addition to the addends here described, other addends for specific purposes. Thus we may add a pour point depressor such as naphthalenechlor wax condensation product, a viscosity index improver such as certain resins or polymerized hydrocarbons and sulfur or phosphorus-containing inhibitors, in addition to our tin compounds. Furthermore, various other metallic compounds may be added to the blend without interfering with the action of our ingredients. Indeed, in some cases it is advantageous to combine with our tin compounds in a hydrocarbon oil blend such materials as calcium dichlorstearate, chromium olate, aluminum stearate, and other metallic soaps. Various halogenated oxygen-bearing ring or aliphatic compounds may be added.

Our addends are admirably suited for use in lubricating oils of all types, including those designed for use in automotive crankcases, Diesel oils, and any other oils of lubricating viscosity. Furthermore, our addends are advantageously blended in gasoline and other petroleum fuels either directly or after being blended first in a lubricating oil and then added to the fuel. Soap-thickened lubricants of all types ranging from those showing only a slight increase in viscosity over that of the mineral oil alone to the semisolid and solid greases containing fifty per cent or more of soap are amenable to treatment according to our invention. The ordinary soaps used in making greases may be replaced in whole or in only small part by some of our tin compounds. We may use up to 30 or 40 per cent of our tin compounds. These addends modify considerably the tackiness, penetration, resistance to breakdown by working or heat, and other properties of the greases. In making these greases, the usual soaps such as sodium stearate, aluminum stearate, calcium soaps of beta fat, and the like may be used to form the large part of the necessary soap. Various other thickening ingredients or materials for other purposes may be added. These include yarn, hair, graphite, glycerol, water, lampblack, mica, zinc dust, litharge, and the like.

The following examples of blends of our addends are given as illustrations and not as limitations:

#### Example 1

| Per cent                                |      |
|-----------------------------------------|------|
| Mid-Continent paraffin base S. A. E. 30 | 99.0 |
| Stannic p-cetyl benzoate                | 1.0  |

#### Example 2

| Per cent                               |      |
|----------------------------------------|------|
| California naphthenic base S. A. E. 30 | 98.7 |
| Stannic p-amyloxybenzoate              | 1.3  |

#### Example 3

| Per cent                                  |      |
|-------------------------------------------|------|
| Pennsylvania paraffin base S. A. E. 10    | 99.4 |
| Stannic tributylphenylacetate             | 0.1  |
| Naphthalene-chlorwax condensation product | 0.5  |

*Example 4*

|                                                  | Per cent |
|--------------------------------------------------|----------|
| Paraffin base bright stock                       | 58.0     |
| Paraffin base neutral oil                        | 40.0     |
| Sulfurized methyl esters of corn oil fatty acids | 0.1      |
| Stannic p-lauroylbenzoate                        | 0.2      |
| Calcium dichlorostearate                         | 1.3      |
| Diphenyl-chlorowax condensation product          | 0.4      |

*Example 5*

|                             | Per cent |
|-----------------------------|----------|
| Naphthenic base S. A. E. 30 | 98.0     |
| Stannic phenylstearate      | 1.3      |
| Methyl dichlorostearate     | 0.7      |

*Example 6*

|                               | Per cent |
|-------------------------------|----------|
| Castor oil                    | 98.3     |
| Sulfurized soy bean oil       | 0.2      |
| Stannic-o-butyrophenylacetate | 1.0      |
| Chlorodiphenyl                | 0.5      |

*Example 7*

|                                         | Per cent |
|-----------------------------------------|----------|
| Mid-Continent paraffin base S. A. E. 40 | 93.8     |
| Voltolized corn oil                     | 5.0      |
| Chlorodiphenylene oxide                 | 1.0      |
| Stannic phenylstearate                  | 0.2      |

It will be obvious that we prefer the stannic of the tin salts as addends to lubricants. In general the stannic salts are more soluble in hydrocarbon oils than the stannous salts. It has even been suggested that some of the acids represented in these salts be added to the blends of the stannous salts to increase the solubility of the salts; however we prefer to avoid the use of free acids because of their corrosive action on certain metal parts being lubricated, especially copper-lead and cadmium-silver bearings. The free acid is not necessary with the stannic salts. We believe the stannic salts are more

soluble in hydrocarbon oils due to the higher content of organic radicals in the salt. We have also found that the stannic salts are more effective anti-oxidants and have more ability to reduce ring sticking.

It will be understood that certain features and subcombinations may be employed without reference to other species or combinations. This is contemplated by and is within the scope of our claims. It is further obvious that various changes may be made in details within the scope of our claims without departing from the spirit of our invention. It is therefore to be understood that our invention is not to be limited to the details described.

Having thus described our invention, we claim:

1. A lubricant comprising a major proportion of an oil of lubricating viscosity and a minor proportion of a stannic salt of an organic acid bearing at least one aromatic ring.
2. A lubricant comprising a major proportion of an oil of lubricating viscosity and a minor proportion of a stannic salt of an organic acid containing both aromatic and aliphatic radicals.
3. A lubricant comprising an oil of lubricating viscosity and from 0.001 to 5 per cent of a stannic salt of an organic acid bearing at least one aromatic ring.
4. A lubricant comprising a major proportion of an oil of lubricating viscosity and a minor proportion of stannic phenylstearate.
5. A lubricant comprising a major proportion of an oil of lubricating viscosity and a minor proportion of stannic p-lauroylbenzoate.
6. A lubricant comprising a major proportion of an oil of lubricating viscosity and a minor proportion of stannic tributylphenylacetate.

BERT H. LINCOLN.  
GORDON D. BYRKIT.  
WALDO L. STEINER.

CERTIFICATE OF CORRECTION.

Patent No. 2,288,289.

June 30, 1942.

BERT H. LINCOLN, ET AL.

It is hereby certified that error appears in the printed specification of the above numbered patent requiring correction as follows: Page 1, second column, line 32, for "slugs" read --sludge--; page 2, second column, line 65, for that portion of the formula reading "CH<sub>3</sub>" read --CH<sub>2</sub>--; and that the said Letters Patent should be read with this correction therein that the same may conform to the record of the case in the Patent Office.

Signed and sealed this 13th day of October, A. D. 1942.

Henry Van Arsdale,  
Acting Commissioner of Patents.

(Seal)